

# UNITED STATES PATENT OFFICE.

AMBROSE G. FELL, OF NEW YORK, N. Y.

## PROCESS OF MAKING LEAD OXID.

SPECIFICATION forming part of Letters Patent No. 674,031, dated May 14, 1901.

Application filed March 30, 1900. Serial No. 10,844. (No specimens.)

*To all whom it may concern:*

Be it known that I, AMBROSE G. FELL, a citizen of the United States, residing in the city, county, and State of New York, have invented certain new and useful Improvements in the Manufacture of Lead Oxid, of which the following is a specification.

This invention relates to the treatment of lead ores and compounds of lead not ores, but of a similar composition, and has for its object to provide a process whereby such ores and compounds may be commercially treated at a reasonable cost for the production of lead oxid for use in the arts and sodium sulfate where the lead ore or lead compound treated contains sulfur, as is usually the case.

The several steps constituting the process which forms this invention may be briefly and broadly stated as follows:

20 First. The treatment of the lead ore or compound by means that will be hereinafter described for rendering the resultant lead salt decomposable by an alkali.

Second. The treatment of the resultant salt of the first step with a free alkali and with the aid of heat for the conversion of as large a percentage of the lead as possible into oxid.

Third. The treatment of the resultant of the second step with water and heat to dissolve out the soluble salts and the separation of said salts by crystallization or otherwise as a by-product.

Fourth. The treatment of the residue from the third step of the process, mainly lead oxid, with a hot aqueous solution of an alkali of sufficient strength to dissolve the oxid, decanting or drawing off the solution from the insoluble residue, and the separation of the oxid from said solution by crystallization.

40 As galena (native lead sulfid) is the most abundant source of lead, the treatment of this ore according to the present invention will now be described, premising that this description gives the preferred method of treatment, which is subject to considerable variation without departing from my invention.

First step: In order to convert the galena into lead sulfate, it is first reduced to powder and then intimately mixed with a suitable quantity of some sufficiently refractory material, also in powder, such as lead oxid, lime, magnesia, &c. This mixture is carefully

heated with access of oxygen, so as to oxidize both the lead and sulfur of the ore. This heating will convert the lead in the charge treated 55 wholly or partially into lead sulfate. The time required for effecting this operation will be only about one hour, and the temperature to which the charge is subjected may vary from 600° to 750° Fahrenheit. It is preferred 60 in this step of the process to employ as a sufficiently refractory material for admixture with the galena about an equal quantity, by weight, of the impure lead oxid, such as is produced at one stage in this process. This 65 refractory material, mixed with the ore, serves mechanically to separate the particles of the sulfid and afford access for the oxygen from the air. It prevents agglomeration, it shortens the time required for this treatment, and it 70 also appears to act chemically when lead oxid is used in first combining with the oxygen from the air and then imparting the oxygen to the sulfid. It also combines with a portion of the sulfuric acid produced, whereby the 75 resultant of the treatment is a basic lead sulfate in lieu of a neutral sulfate. The former is preferable for the subsequent treatment by this process.

Second step: The treatment of the ore as 80 described in the first step of the process renders it decomposable by an alkali, and the second step relates to such decomposition. The product of the first step is cooled, by preference, and dry caustic soda in powdered form 85 is thoroughly mixed therewith, the proportion of the alkali being about equal to its combining equivalent with the sulfur of the sulfid treated, which for practical operations would be about twenty-six pounds of the 90 finely-powdered caustic soda to one hundred pounds of crude galena, which is the sulfid commonly treated. If the soda is not finely powdered, it is well to pass the whole mass through a mill which will serve both to grind 95 and mix it. This mixture is submitted to heat, and the soda almost immediately converts the oxidized sulfur compounds into lead oxid and sodium sulfate; but in practice the mass is preferably stirred for about thirty 100 minutes after being submitted to heat. The decomposition which follows the addition of the alkali will be furthered or accelerated by the presence of the elements of water. This

addition can be effected by introducing steam into the mass during the oxidation of the lead compounds, or the alkali may be moistened with water or steam. The employment of 5 steam or water, as described, is not, however, necessary to the operation.

Third step: The product of the second step, which is mainly lead oxid mixed with some undecomposed ore, matrix, and the sodium 10 sulfate formed by the combination of the sulfur and oxygen with the soda, is now put into a suitable vessel—say an iron tank adapted to be heated with steam—and water is added to dissolve out the soda salts therein. The 15 temperature at which this is effected is not important. Stirring facilitates the solution of the salts. The mixture is allowed to settle and the solution is decanted or drawn off from the insoluble residue and allowed to 20 cool. If the solution be strong enough, the sodium sulfate will crystallize out and forms a by-product of the process. To avoid the necessity of the concentration of the solution and to assure its strength, a solution of sodium sulfate may be employed in this step in 25 lieu of water.

Fourth step: The undissolved residue remaining in the tank is next treated with a strong solution of caustic alkali, preferably 30 soda. In practice this solution is made by dissolving one hundred pounds of caustic soda in about two hundred pounds of water. The 35 solution used should contain an amount of soda equal to three or four times that of the weight of the lead oxid contained in the mixture under treatment; but considerable variation in the strength of the solution is permissible. If it be too weak, the oxid will not precipitate on cooling and the solution 40 will require concentration. Potash or other caustic alkali may be employed in lieu of soda; but as soda is satisfactory and affords a marketable by-product it is preferred. The mixture is heated to about the boiling-point, and the mass therein will be stirred, 45 by preference. All of the lead oxid will be dissolved, and after this is effected the steam is shut off and the undissolved matter allowed to settle. The clear solution of lead 50 oxid is now drawn off into a vessel containing metallic lead in such form as to present as much surface as possible. In practice granulated or sponged lead, formed by pouring molten lead into water, is employed. The 55 hot solution of lead oxid is allowed to remain in this vessel in contact with the metallic lead for a short time and is then drawn off into another vessel to cool, and as it cools it deposits the oxid in the form of crystals. These 60 latter will vary somewhat in size and color, according to the strength and volume of the solution and the time taken up in cooling. When the cool and clear solution of soda is drawn off from the oxid, the latter is washed 65 to free it from alkali, dried, and is then ready for use in the arts.

The solution of the caustic soda employed

for dissolving out the lead oxid may be used almost indefinitely with very little loss; but the submission of the solution while hot to 70 contact with metallic lead constitutes a very important feature of the process, as it preserves the usefulness of the soda solution as a permanent solvent of the lead oxid and secures the production of a pure lead protoxid instead of a mixture of various oxids. 75 Ordinarily a caustic-soda solution may be employed with good results four or five times only as a solvent of the oxid, after which it loses its solvent property. Presumably this 80 is due to its having become gradually charged with an oxid richer in oxygen than the protoxid. This higher oxid will be only sparingly precipitated on cooling the solution, and its presence in quantity prevents the 85 dissolving of the protoxid, which latter precipitates much more readily. To obviate the great loss of soda which such a condition of the soda solution would entail, the hot solution before the precipitation of the protoxid 90 is filtered through or put in contact with the spongy lead, as before described. The action of the metallic lead is to reduce the higher oxids, such as peroxid and red lead, to protoxids by combining with their excess of oxygen. 95 Thus the lead oxids are practically all precipitated and the usefulness of the soda solution as a solvent is permanently maintained.

The sponged lead may be placed as a filtering material in a steam-jacketed tank and the hot solution be passed through the said tank on its way to the cooling and precipitating vessel. By this arrangement the sponged lead may serve as a mechanical filter also. 100

It is not important that the soda or other alkaline solvent shall be pure or free from admixture with other substances, such as the sulfates, chlorides, and carbonates of the alkali employed. So long as there is enough of the 110 free caustic alkali present to effect the solution of the lead oxid it will suffice. Thus it follows that instead of employing the commercial caustic soda the carbonate, as "soda-ash," may be employed, and by treatment of 115 this with lime in a known way it may be rendered caustic wholly or in part and will thus serve the purposes required in this process.

The first step of this process, as described, is much preferred over the ordinary slow and expensive mode of roasting the lead ore; but nevertheless the old or known mode of roasting may be used in connection with the last three steps of this process, although not of course to such good advantage nor with such 125 good results. It will be understood that the term "refractory" as applied to the material mixed with the lead compound in the first step of the process is relative and means only sufficiently refractory for the purpose. The 130 lead oxid, for example, is sufficiently refractory to resist the heat employed.

Native lead sulfate may be treated by this process, in which case the first step would

obviously be omitted, or native lead carbonate may be treated in the same manner as the sulfate, in which case, however, the salt of the alkali produced would be a carbonate instead of a sulfate.

Having thus described my invention, I claim—

1. The herein-described process of treating lead ore or similar lead compounds, which consists in first converting the lead into a lead salt decomposable with an alkali, then treating the mass with an alkali to convert the lead into oxid, then dissolving out the soluble salts of the alkali, then heating the residue containing lead oxid with a solution of alkali to dissolve the lead oxid, and then cooling said solution to allow the oxid to crystallize out.
2. The herein-described process of treating lead sulfid, which consists in first converting the sulfid into a lead salt decomposable with an alkali, then mixing the mass with finely-powdered alkali, then heating the mixture to convert the lead into oxid, then dissolving out the sulfate of the alkali from the mass, and finally treating the residue with a solution of caustic alkali to dissolve and remove the lead oxid, substantially as set forth.
3. The herein-described process, which consists in heating a mass containing lead oxids with a solution of caustic alkali to dissolve the oxids, then reducing the higher oxids in the solution to protoxid, and then separating the protoxid, substantially as set forth.
4. The herein-described process of treating a mass containing lead oxid, which consists in heating the mass with a solution of caustic alkali to dissolve the oxid, then, while hot, putting said solution in contact with metallic lead to decompose the higher oxids, and then cooling the solution to permit the oxid to crystallize out, substantially as set forth.

5. The herein-described process of treating lead sulfid, which consists in mixing the powdered sulfid with a powdered suitably refractory material and heating the mass with access of oxygen to convert the sulfid into sulfate, then heating the mass with soda to convert the lead into oxid, then dissolving out the sodium sulfate, then heating the residue, containing lead oxid, with an alkaline solution to dissolve the lead oxid, then cooling said solution to allow the oxid to crystallize out, and then drying the oxid, substantially as set forth.

6. The herein-described process of treating lead sulfid, which consists in mixing the powdered sulfid with a powdered suitably refractory material and heating the mass with access of oxygen to convert the sulfid into sulfate, then heating the mass with an alkali to convert the lead into oxid, then dissolving out the sulfate of the alkali, then heating the residue, containing lead oxid, with an alkaline solution to dissolve the lead oxid, then cooling said solution to allow the oxid to crystallize out, and then drying the oxid, substantially as set forth.

7. The herein-described method of treating lead sulfid, which consists in mixing it with lead oxid, both in pulverized form, then heating the mass with access of oxygen, to convert the lead of the sulfid into sulfate, then heating the mass with an alkali to convert the sulfate into oxid, then dissolving out the sulfate of the alkali, and then dissolving out the lead oxid, substantially as set forth.

In witness whereof I have hereunto signed my name, this 29th day of March, 1900, in the presence of two subscribing witnesses.

AMBROSE G. FELL.

Witnesses:

THOMAS M. FELL,  
PETER A. ROSS.